

No. 642,320.

Patented Jan. 30, 1900.

G. W. GESNER.

PROCESS OF PRODUCING ALLOYS OF HYDROGEN AND IRON.

(Application filed May 2, 1899.)

(No Model.)

2 Sheets—Sheet 1.



Witnesses

M. F. Boyle  
J. B. Clautice

Inventor:

G. W. Gesner  
By Thomas Drew Gleason  
Attorney

No. 642,320.

Patented Jan. 30, 1900.

G. W. GESNER.

PROCESS OF PRODUCING ALLOYS OF HYDROGEN AND IRON.

(Application filed May 2, 1899.)

(No Model.)

2 Sheets—Sheet 2.

Fig. 4.



WITNESSES:

*Q. C. Vining*

*J. B. Clautice*

INVENTOR

*Geo. W. Gesner*  
BY

*James Drew Stetson*  
ATTORNEY

# UNITED STATES PATENT OFFICE.

GEORGE W. GESNER, OF NEW YORK, N. Y.

## PROCESS OF PRODUCING ALLOYS OF HYDROGEN AND IRON.

SPECIFICATION forming part of Letters Patent No. 642,320, dated January 30, 1900.

Original application filed March 10, 1896, Serial No. 582,600. Divided and this application filed May 2, 1899. Serial No. 715,323. (No specimens.)

To all whom it may concern:

Be it known that I, GEORGE W. GESNER, a citizen of the United States, residing in the borough of Brooklyn, in the city and State of New York, have invented a certain new and useful Process of Producing an Alloy of Hydrogen and Iron, of which the following is a specification.

I produce a new alloy composed of a permanent combination of iron and hydrogen adapted to be worked either by forging or by casting. The means by which I produce it induce an absorption of the gas by subjecting extended surfaces of the heated iron to the same and subsequently melting the alloy thus produced.

The alloy possesses extraordinary properties in resisting oxidation and corrosion. It is unaffected even by sulfuric acid or aqua regia. It can be worked in the same manner as iron. The specific gravity is somewhat less, but it possesses nearly the strength of iron.

My experiments indicate that the union of the hydrogen with the iron is stable and will remain under all ordinary or extraordinary conditions to which it may be subjected.

The alloy first formed on the surface of the iron obstructs the action of the hydrogen on the iron within. At this stage it is not strong, and its adhesion to the remainder of the iron is sufficiently weak to allow the thin coatings of alloy to be removed at intervals by sufficiently-violent action. The scales being afterward subjected to heat melt into a single piece which possesses the qualities above defined.

The iron must be previously reduced by puddling or analogous means to the condition of wrought-iron or low steel and rolled thin and coiled or otherwise conditioned to expose a large surface on which to form the thin scales in which the alloy first appears.

The accompanying drawings form a part of this specification and represent what I consider the best means of carrying out the invention.

Figure 1 is a vertical section on the line 1 1 in Fig. 2. Fig. 2 is a horizontal section of a portion on the line 2 2 in Fig. 1. Fig. 3 is a section through a portion of the upright re-

tort on a larger scale, to show a preferable form of the joints. Fig. 4 illustrates an apparatus adapted for the practice of my invention in connection with a blast-furnace. 55

Similar letters of reference indicate corresponding parts in all the figures where they appear.

A is a pipe bringing steam from a boiler. (Not represented.) A' is a series of convolutions in such pipe, heated by a fire in the furnace C to a temperature about 1,500° Fahrenheit.

B is a valve which controls the flow of the steam from the boiler to the convolutions, 65 and D is a second valve which controls the delivery of the contents of the coil into the base of the upright retort.

The effect of the apparatus so far as yet described is to decompose the steam, the oxygen going to line the interior of the coil A' with 70 oxid of iron, while the hydrogen thus liberated moves forward. When the operation is properly conducted, free hydrogen alone in the first part of the treatment and the same 75 with hydrocarbon vapor at a later stage are delivered past the valve D.

It will be understood that the apparatus presents a thick coating of fire-brick or other refractory non-conducting material to withstand the heat and a lining of ganister or other suitable material to maintain the integrity of the interior.

A hydrocarbon-inlet M leads from a vessel, which for convenience may be the small vessel N, at an elevation of about twenty-five feet above the coil A'. In this for each batch of one ton of iron I place one (1) quart of naphtha, about 65° to 70° Baumé, and tightly close the vessel N, the descent of the naphtha being controlled by a cock C.

P is an upright retort composed of lengths of fire-clay matched together and having the lower end sealed with water in a concave tank Q. The interior of this upright passage, which I have termed a "retort," is smooth and slightly tapered, the large end downward. The upper end is open to the atmosphere. A considerable length of this retort is enveloped in a furnace T, which maintains a high temperature in all that part of the retort above the plane of the furnace-bars T' and in the

quantity of iron moving slowly downward therein and in the hydrogen moving upward in the interstices. Thus conditioned the hydrogen is absorbed nearly uniformly by all the surfaces of the iron. Thin sheet-iron in rolls or other convenient form is fed in at proper intervals at a door *p* near the top, and the iron emerges at the bottom below the surface of the water seal in the tank *Q* and is hauled up the inclined sides of the tank by hand or by machinery, and its place is supplied by more descending from above in the smooth interior of *P*, so that the operation is continuous.

15. The steam-pressure in the convolutions is maintained at about forty pounds, except for a short period. After the operation is continued about two hours the valve *B* is so far closed that the pressure in the convolutions is lowered to about ten pounds per square inch and the cock *C* is opened, allowing the naphtha to descend through the pipe *M* and enter the coil *A'*. This condition is maintained for about twenty minutes, when the naphtha will be found to have nearly or quite all descended. Now the cock *C* is closed and the valve *B* is again set wide open, restoring the full steam-pressure in the apparatus, and this condition is maintained for forty minutes, or until the end of the operation. The entire treatment will occupy about three hours under ordinary conditions. The heated iron descending through the bath of hydrogen in this, which I term the "coating process," absorbs the hydrogen and forms my alloy in a crude condition. As nearly as I have been able to determine, aided by a great number of small experiments, the temperature should be about 1,800° Fahrenheit. The alloy is now in the form of a scale on the surfaces of the sheet-iron. If allowed to continue a long time, the sheet-iron will be alloyed quite through; but the operation will proceed more slowly after the iron is covered 40 with a coating of alloy. The alloy at this stage is not strong, and it may be beaten off from the core of unalloyed iron remaining by subjecting the coated iron to violent concussions in a common agricultural threshing-machine or analogous apparatus, and the detached scale being collected by a process which may be analogous to winnowing the scaled iron may be again treated until alk is made to absorb its proper equivalent of hydrogen and is thus transformed into the scales of alloy. Finally, the scales are heated to a temperature a little below that of ordinary melted iron. At this temperature it is melted, and the several scales unite in a 55 fluid or semifluid state, and the semiliquid matter may be cast in sand or in solid molds like iron or steel.

60. The structural character of my alloy may be changed by subsequent treatment. For instance, it may be reheated and mechanically worked to acquire the laminated or fibrous character of wrought-iron.

I ascribe to the treatment with naphtha at one period an important duty in absorbing and carrying away any oxygen which may by any chance be present in the alloy.

Modifications may be made within the scope of the claims without departing from the principle or sacrificing the advantages of the invention.

It will be understood that the treatment of the steam in the convolutions *A'* of the pipe *A* is the mode which I consider most desirable for producing hydrogen from steam in the liberal quantities and at the pressures required. The interior of the convolutions *A'* may be subsequently deoxidized by flowing a hydrocarbon through the same at a proper temperature, as has long been practiced by myself and others. The surface of iron exposed may be increased by any ordinary or suitable devices, as the filling of the convolutions *A'* loosely with scrap-iron. The hydrogen for my treatment may be produced by other means than by the decomposition of steam. Hydrogen produced by any available means may be used to produce my alloy by this process.

I can treat ores of iron and produce my alloy at the same time that the iron is reduced from the ore to the metallic state. To effect this, I use a non-heat-conducting vessel, with provisions for admitting a gaseous blast and for discharging the finished product, charging it with fuel, iron ores, and flux in the proportions indicated by the chemical composition of each. The form of the apparatus may be that of an ordinary blast-furnace *V*, as shown in Fig. 4. In such case I treat the ore first with the ordinary blast, which can enter at any convenient place and at a certain time, determined by the progress of the reduction of the ores to the metallic state. I cut off the air-blast and substitute hydrogen from the convolutions *A'* by closing a valve *W*, controlling the induction of air, and opening the valve *D* and continuing its application about two hours in the same manner as before described. The slag and the alloy are drawn from the smelter by the tap.

All iron ores and all manufactured iron contain silicon, alumina, &c., in varying quantities, and consequently more or less of chemically-pure iron proportionately, and all and every kind can be used in the production of the alloy. Therefore any given charge of the alloy will contain more or less hydrogen in proportion to the purity of the iron that has been used, and any sample from any such charge will yield more or less hydrogen on analysis.

As the result of analysis of different samples of the alloy I state that as a fair average eleven one-hundredths of one per cent. of hydrogen, by weight, are found in the alloy. At this average the amount of combined hydrogen in one ton of two thousand pounds of the alloy would yield eighty-two and one-half pounds of water containing gaseous hydrogen equiva-

lent to two thousand two hundred cubic feet, temperature 60° Fahrenheit, barometer 30.

It is important that the scales or the small thickness of iron saturated with hydrogen 5 from the surface in what I have termed the "coating process" be melted. To shape the article in iron, wrought or cast, and then treat it with heat and hydrogen until it is saturated throughout its entire thickness, will not produce 10 my alloy nor any useful approach thereto by reason of the crumbly and weak condition which obtains in the mass. The alloy must be melted in order to attain a sound and strong condition of the metal, so as to realize 15 any considerable portion of the benefit of my invention.

I use the word "iron" to include all the grades of iron and steel.

I do not in this patent claim the alloy thus 20 formed, such being the subject of a separate patent, for which application was filed March 10, 1896, Serial No. 582,600, of which the application for the present patent is a division.

I claim as my invention—  
25 1. The process described of producing a

fusible alloy of iron and hydrogen by first puddling the iron, subsequently reducing it to a form presenting a greatly-extended surface, heating such iron in the presence of free hydrogen and allowing time for the latter to 30 be absorbed, and subsequently detaching and melting the scale thus produced, substantially as herein specified.

2. The process described of producing a malleable alloy of iron and hydrogen by first 35 puddling the iron, subsequently reducing it to a form presenting a greatly-extended surface, heating such iron in the presence of free hydrogen and allowing time for the iron to absorb the hydrogen, subsequently detaching 40 and melting the scale thus produced and again mechanically working such alloy, substantially as specified.

In testimony that I claim the invention above set forth I affix my signature in presence of two witnesses.

GEORGE W. GESNER.

Witnesses:

M. F. BOYLE,  
J. B. CLAUTICE.